# EUROPEAN PATENT SPECIFICATION

(11) **EP 0 372 800 B1**
(45) Date of publication and mention of the grant of the patent: **06.03.1996**
(21) Application number: 89312373.7
(22) Date of filing: 28.11.1989
(51) Int. Cl.: B41M 5/38

(54) **Manufacturing method for a heat-sensitive transfer recording material**
Verfahren zur Herstellung eines wärmeempfindlichen Übertragungsaufzeichnungsmaterials
Méthode pour la fabrication d' un matériau d'enregistrement par transfert thermique

(30) Priority: 02.12.1988 JP 305187/88; 02.12.1988 JP 305311/88; 06.12.1988 JP 308596/88; 06.04.1989 JP 87723/89
(43) Date of publication of application: 13.06.1990
(73) Proprietor: KONICA CORPORATION, Tokyo 160 (JP)
(72) Inventor: Koshizuka, Kunihiro, Hino-shi Tokyo (JP); Abe, Takao, Hino-shi Tokyo (JP)
(74) Representative: Brock, Peter William

(56) References cited:
- EP-A- 0 249 195
- GB-A- 2 044 473
- PATENT ABSTRACTS OF JAPAN vol. 12, no. 164 (M-698)(3011) 18 May 1988, & JP-A-62 280084 (DAINIPPON PRINTING COMPANY LIMITED) 04 December 1987
- PATENT ABSTRACTS OF JAPAN vol. 14, no. 13 (M-918)(3956) 11 January 1990, & JP-A- 01 258989 (UNION KEMIKAA K.K.) 16 October 1989,

## Description

### FIELD OF THE INVENTION

This invention relates to a heat-sensitive recording material and, more particularly, to a heat-sensitive recording material capable of forming an excellently long-lasting printed-image, stably, simply, efficiently, and inexpensively.

### BACKGROUND OF THE INVENTION

In recent years, a heat-sensitive color-developing paper has come into wide use, as a heat-sensitive recording material for a facsimile.

Such a heat-sensitive color-developing paper as mentioned above usually forms a printed-image thereon in the manner that the paper surface is so heated as to color-develop the heated portion thereof.

The above-described heat-sensitive color-developing papers have had the problems so far that the surface thereof is liable to be discolored by the change on standing after an image is printed and, in particular, that the storage-stability of a printed-image has been deteriorated, for example, the portion other than the printed portion has also been color-developed as same as in the printed portion, when the portion other than the printed portion has been exposed repeatedly to heat or light.

On the other hand, a heat-sensitive transfer-paper has been proposed to serve as a heat-sensitive material having an excellent storage-stability.

Ordinarily, such a heat-sensitive transfer paper comprises the two components, namely, an image-tranfer-recipient paper and a heat-transfer member, each arranged independently. In this ordinary case, the two components are stored in a rolled form, laid one upon another or separated one from another. When using this type of heat-sensitive transfer-paper, a printed-image may be formed on the transfer-image-recipient paper in such a manner that a colorant containing layer of the heat-transfer member is heated to fuse and the heat-transfer member is then brought into pressure-contact with the transfer-image recipient paper, so that an image in the portion to be transferred may be transferred to the image-recipient paper.

Such a heat-sensitive transfer-paper, different from heat-sensitive color-paper, requires two composing materials (transfer recipient paper and heat transfer material) in order to get a recording paper having printed images. Therefore, it has such problems as that, for example, control and check must be needed for both of transfer recipient paper and heat transfer material, as the heat-transfer material is composed of support and a colorant containing layer and the foregoing support becomes completely useless after being printed so that the cost of heat transfer material is expensive, as originally the transfer recipient paper and the heat transfer material are separated and the heat transfer material is a thin sheet so that wrinkles are easy to be made on transfer recipient paper and heat transfer material when printing is done while rolled heat-sensitive transfer paper is wound therefore it is liable that printing order goes out of order, troubles occur in winding operation of heat-sensitive transfer paper or running of heat-sensitive transfer paper cannot be done stably.

As a commonly-used heat-sensitive recording material, an ink ribbon having a thermosoftening colorant containing layer on a support is used. In the case of this ink ribbon, the foregoing ink ribbon is contacted to the transfer recipient material, for example paper, and heat is applied imagewisely so that a heat-fusing thermosoftening colorant layer is transferred onto a recording material to form a printing image thereon.

In this ink ribbon, too, the support becomes useless after being printed. Therefore, the cost of the ink ribbon is expensive.

Besides, on the other hand, the foregoing heat-sensitive transfer paper or the foregoing heat-sensitive color-developing paper are used as barcode use or label use. In these cases, not only image preservation but also abrasion resistance becomes a problem. If the foregoing heat-sensitive transfer paper is used, abrasion resistance is bad, and if the foregoing heat-sensitive color-developing paper is used, both of image preservation and abrasion resistance are bad.

EP-A-0 249 195 describes a thermal transfer recording method. A thermal transfer recording material comprising a support carrying a first and a second ink layer is placed in contact with a image receiving layer carried by a separate support. Energy is applied imagewise to the transfer material, e.g. by means of a thermal printer head, causing the ink layers to adhere imagewise to the image receiving layer. The two supports are peeled apart after a critical time interval to provide a transfer image on the supported image receiving layer.

JP-A-62 280 084 describes a method of making a thermal transfer ink sheet which can be laminated to an image receiving sheet to form a recording paper for use in thermal recorders and facsimile apparatus in place of heat-sensitive paper. After recording the two sheets are peeled apart.

JP-A-1 258 989 discloses a thermal transfer ink sheet prepared by laminating an image receiving sheet with a thermally sensitive colorant layer.

### BRIEF DESCRIPTION OF THE DRAWINGS

Figs. 1 to 6 are each the illustrations of the principle applied to the invention; Fig. 7 is a cross-sectional illustration of one of the embodiments of the invention; Fig. 8 is a cross-sectional illustration of the substantial functions of the recording material shown in Fig. 7; Fig. 9 is a cross-sectional illustration of another embodiment of the invention; Fig. 10 is a cross-sectional illustration of the substantial functions of the recording material shown in Fig. 9; Fig. 11 is a cross-sectional illustration of a further embodiment of the invention; Fig. 12 is a cross-sectional illustration of the substantial functions of the recording material shown in Fig. 11; Fig. 13 is a cross-sectional illustration of a still further embodiment of the invention; Fig. 14 is a cross-sectional illustration of the substantial functions of the recording material shown in Fig. 13; Fig. 15 is an illustration of the first embodiment; Figs. 16 through 26 are each the cross-sectional illustrations of the other embodiments of the invention; Fig. 27 is an illustration of the second embodiment; Figs. 28 to 35 are each the several alternative embodiments of the heat-sensitive materials of the invention; and Fig. 36 is an illustration of the third embodiment; wherein
1 ... Image-receiving layer; 2 ... Colorant layer; 5 ... Heat-sensitive material; 6 ... Support; 6a ... Transparent support; 7 ... Thermosoftening colorant layer; 7b ... Special thermosoftening colorant layer; 8 ... Sublayer; 9 ... Thermosoftening layer; 10 ... Peelable layer; 11 ... Peeling-supporting layer; 12 . Antifogging layer; 13 ... Release layer; 14 ... Dye; 15 ... Dye-supplying layer; 16 ... Mordant layer; 17 ... Sublayer for masking; 18 ... Adhesive mordant layer; 18a ... mordant layer; 18b ... Adhesive mordant layer; 20 ... Adhesive layer; 19a ... dye-supplying layer; 19b ... Adhesive dye-supplying layer; and 21 ... Antifogging layer

### DETAILED DESCRIPTION OF THE INVENTION

According to the present invention there is provided a method of making a heat sensitive transfer recording material for use in a heat sensitive transfer recording system, comprising forming an image receiving layer and providing thereon, a colorant layer containing a colorant and a binder, wherein the image receiving layer is adhered to the colorant layer so firmly that the image receiving layer can be separated from the colorant layer with a peeling force, measured in accordance with JIS 6854, of 0.1 to 1000 g/mm at an angle of 180° after forming an image on the image receiving layer, said method being characterised by comprising (a) preparing a coating composition comprising said colorant and said binder, (b) coating said coating composition on to said image receiving layer, and (c) drying the coated composition to form said colorant layer.

In the invention, as shown in Figure 1, generally speaking, image is formed on the foregoing image receiving layer in the heat-sensitive recording material comprising the foregoing image receiving layer 1 and colorant containing layer 2.

Namely, in this image forming mechanism, when heat is added image-wisely to the surface of the image receiving layer 1 not contacting the colorant containing layer 2 (in Figure 1, heat is added from arrow mark direction A), or when heat is added image wisely to the colorant containing layer 2 not contacting the image receiving layer 1 (in Figure 2, heat is added from arrow mark direction B), stronger adhesive power is generated to the heated part in the colorant containing layer 2 against the image receiving layer 1. Then, when the colorant containing layer 2 is detached from the image receiving layer 1, the colorant containing layer 2 to be heated is coagulated and broken as shown in Figure 2, or it is surfactantly destroyed. As a result, colorant containing part 3 separated from the detached colorant containing layer 2 remains on the image receiving layer 1, so that layer 1 having this image is utilized as an image recording body.

On the other hand, as shown in Fig. 4, in case that the moving speed of colorant in the colorant containing layer 2 is big, when heat is added image-wisely, the colorant of the colorant containing layer 2 is heat-shifted with a binder to the heat image receiving layer 1 side, and in the colorant containing layer 2, the colorant near the surface of the colorant containing layer 2 is moved to the image receiving layer 1 side. As a result, in the colorant containing part 3 remaining on the image receiving layer 1 after the colorant containing layer 2 is detached, as shown in Fig.5, an image receiving layer 1 is formed wherein colorant containing layer 2 has no or little colorant on its surface part 4.

In another image forming mechanism, the heat recording material of the invention is the material where an image receiving layer 1 is superimposed on a colorant layer 2 comprising a colorant 3 diffusable by heat energy and a binder.

And when heat is applied imagewisely to the surface of the image receiving layer 1 not contacting the colorant containing layer 2 (in Fig.6, heat is added from arrow mark direction a) or when heat is added imagewisely to the colorant containing layer 2 not contacting the image receiving layer 1 (in Fig. 6, heat is added from arrow mark direction b), stronger adhesive power is generated to the heated part in the foregoing colorant containing layer 2, at the same time, colorant in the colorant containing layer is difused and moved into the image receiving layer 1. And when the image material containing layer 2 is peeled off the image receiving layer 1, an image receiving layer 1, image receiving layer 1 can be obtained so as to have an image formed thereon by transferring a colorant i.e., a dye, with a heat-diffusion, from heated colorant-containing layer 2 into image-receiving layer 1. An image receiving layer having this image can be used as an image recording body. Besides, when the colorant containing layer is peeled off from the image receiving layer, in case that colorant containing layer is coagulated and destroyed, a part of colorant containing layer remains on the surface of image receiving layer having an image. So, the remaining colorant containing layer has a role of protective layer so that an image excellent in abrasion resistance can be formed.

Heat-sensitive recording material in the invention is not limited to the double-layer structure composed of the foregoing image receiving layer and colorant containing layer so that various kinds of layer structures can be adopted within the range that they do not interfere the objects of the invention. For example, heat-sensitive recording material of the invention can also have such an appropriate layer arrangement as is comprised of a release layer, a peelable layer, a supporting layer for the peelable layer, a supporting layer, an adhesive layer, and an antifogging layer.

The heat sensitive recording material of the invention is a heat sensitive recording material where an image receiving layer is adhered directly or indirectly to a colorant layer so firmly that the image receiving layer can be separated from the colorant layer with a peeling force of 0.1 to 1000 g/mm at an angle of 180° after forming an image on the image receiving layer. The heat sensitive recording material of the invention excludes a heat sensitive recording material where an image receiving layer is simply superposed directly or indirectly onto a colorant layer. The peeling force is measured by the method as described in JIS 6854.

Now, an appropriate embodiment of the invention will be detailed below.

### -The first embodiment-

The first appropriate embodiment of the invention is the foregoing heat-sensitive recording material wherein the foregoing image receiving layer is a support and the foregoing colorant containing layer is a thermosoftening colorant layer.

### (1) Basic structure

As shown in Figure 7, heat-sensitive recording material 5 having the basic structure of the first embodiment is formed by piling a thermosoftening coloring layer 7 as a colorant containing layer on the support 6.

The foregoing support is preferable to have a good heat resistance and dimensional stability.

As the materials of the support; papers such as plain paper, condenser paper, laminated paper, and coated paper; resin films such as those made of polyethylene, polyethyleneterephthalate, polystyrene, polypropyrene, or polyimide; composite materials of paper and resin film; and metal sheets such as that made of an aluminium foil.

Such supports are used as a recording member supporting an image, so that it may be necessary to have an enough self-supportability. In order to satisfy it, the thicknesses of the supports are to be regulated to not more than 500 µm, for example, and, preferably, within the range of 1 to 200 µm. If the thickness of such a support is less than 1 µm, there may be a possibility to lose the self-supportability of the support.

The forms of the supports can be so suitably determined as to meet the purposes of the heat-sensitive recording material they can be taken in any desirable forms of, for example, a tape, a sheet, and a label.

Between the support and the thermosoftening type colorant layer, an adhesive layer may be interposed to strengthen the adhesivity of the thermosoftening type colorant layer to the support.

Such an adhesive layer, as mentioned above, can be formed normally with the conventional compositions used as adhesives.

As an example of such adhesives, a hot-melting adhesive may be given. It is a composition comprising a resin such as an ethylene-vinyl chloride copolymer, wax, plasticizer, tackifier, antioxidant, and fillers.

Therefore, as an example of compositions composing an adhesive layer, a composition comprising an ethylene-vinyl chloride copolymer, wax, plasticizer, tackifier, antioxidant, filler, and colorant may be given.

Besides, they include the compositions such as those composing a polyvinyl acetate emulsion type adhesive, those composing a chloroprene type adhesive, those composing an epoxy resin type adhesive, each can be used as the compositions for composing an adhesive layer.

The adhesive composition includes, for example, natural rubber, chloroprene rubber, butyl rubber, polyacrylic acid esters, nitrile rubber, polysulfides, silicone rubber, SBR, Polyisoprene, Polyvinylether and Buna N.

The thickness of reclaimed rubber, in such an adhesive layer is within the range of, normally, 0.1 to 30 µm and, preferably, 0.3 to 10 µm.

The foregoing thermosoftening colorant layer contains binders and colorants.

As the binders, heat-fusible substances and a thermoplastic resins may be included as examples.

The typical heat-fusible substances include, for example; vegitable wax such as carnauba wax, Japan wax, ouricury wax, and esparto wax animal wax such as beeswax, insect wax, shellac wax, and whale wax; petroleum wax such as paraffin wax, microcrystal wax, Polyethylene wax, ester wax and acid wax; and mineral wax such as montan wax, ozokerite, and ceresin wax. Besides the above, they further include, for example, higher aliphatic acids such as palmitic acid, stearic acid, margaric acid, and behenic acid; higher alcohols such as palmityl alcohol, stearyl alcohol, behenyl alcohol, margaryl alcohol, myricyl alcohol, and eicosanol; higher aliphatic esters such as cetyl palmitate, myricyl palmitate, cetyl stearate, myricyl stearate; amides such as acetamide, proprionamide, palmitamide, stearamide, and amide wax; and higher amines such as stearyl amine, behenyl amine, and palmityl amine.

The thermoplastic resins include, for example, those of ethylene type copolymers, Polyacetals, polyamides, polyesters, polyurethanes, polyolefins, Polyacrylate, Poly vinyl chloride, celluloses, rosin, ionomer resins, and petroleum; elastomers such as natural rubber, styrene-butadiene rubber, isoprene rubber, chloroprene rubber, and diene copolymers; rosin derivatives such as ester gum, rosin-maleic resin, rosin-phenol resin, and hydrogenated rosin resins such as phenol resin, terpene resin, cyclopentadiene resin, and aromatic hydrocarbon type resin; and these polymer compounds have a softening point of 50 to 200°C, softening point is measured by the ring and ball method as described in JIS K2531.

By suitably selecting the foregoing heat-melting material and thermoplastic material, thermosoftening colorant layer having a desired thermosoftening point or heat-melting point can be prepared.

The colorants include, for example, pigments such as inorganic and organic pigments or dyes.

The inorganic pigments include, for example, titanium dioxide, carbon black, zinc oxide, Persian-blue, cadmium sulfide, iron oxide, and chromates of lead, zinc, barium, and calcium.

The organic pigments include, for example;, those of an azo, thioindigo, anthraquinone, anthanthrone and triphenyl dioxazine; vat dyes/pigments; phthalocyanine pigments such as those of copper phthalocyanine and the derivatives thereof; and quinacridone pigments.

The foregoing dyes include, for example, acid dyes, direct dyes, disperse dyes, oil-soluble dyes, and oil-soluble metal-containing dyes.

The colorant content of the thermosoftening colorant layer is within the range of, usually, 5 to 60% by weight and, preferably, 10 to 50% by weight.

For the above-mentioned thermosoftening colorant layer, the kinds of the binder and colorant, and the compounding amounts thereof, can be determined, provided, the thermosoftening colorant layer may have a self-supportability, and the heat-melting material and thermoplastic material may suitably be selected so as to satisfy the other required physical properties.

The thermosoftening colorant layer is also allowed to contain, besides the above-given components, the other additives such as a wax, surfactant, higher fatty acid derivative, higher aliphatic alcohol, higher aliphatic ether, phosphoric acid ester, and organic or inorganic filler.

When carbon black is selected to use as an inorganic material filler, a 'stone wall' structure is formed by the strong coagulation power of carbon black, and the colorant exuded, by being applied with heat, from the gaps of the 'stone wall' so as to be moved onto the surface of the support. On the other hand, when using alumina particles as an inorganic filler, colorants around the alumina particles are activated sooner by heating, so that the activated colorant moves to the support through between alumina particles by capillary phenomenon with the aid of a thermal expansion phenomenon produced with raising temperature of the colorant. In this way, a thermosoftening colorant layer having a special structure can be formed.

The thickness of the thermosoftening colorant layer can be within the range of, normally, 0.5 to 20 µm and, preferably, 1 to 10 µm so long as the thickness is adjusted so that the colorant layer may be peeled apart from the support and an heat energy may be applied with a well response from the thermosoftening colorant layer's side.

If required, a peelable layer of which will be detailed later may further be provided to improve the peeling property between the thermosoftening colorant layer and the support. It is also allowed to provide an interlayer, and a thermosoftening colorant layer in this order onto the support.

Now, one of the examples of the mechanism for being printed will be detailed. When heat-sensitive recording material 5 shown in Fig. 7 is heated imagewise, for example, by making use of a heating means such as a thermal head, for example, on the surface of the support 6, the thermosoftening colorant layer 7 on the other side becomes melted. As a result, the adhesion of the heated thermosoftening colorant layer to support 6 is greater than that of the thermosoftening colorant layer which is not heated to the support 6. Then, as shown in Fig. 8, when the thermosoftening colorant layer 7 is separated from the support 6, the heated thermosoftening colorant layer is subjected to cohesive failure so that at least a part thereof remains on the support, and the thermosoftening colorant layer which is not heated is separated from the support without remaining on that. Therefore, when the thermosoftening colorant layer is separated from the support, the heated thermosoftening colorant layer remains on the support, whereby an image is formed on it. As shown in Fig. 8. the thermosoftening colorant layer of the recording material of the invention is subjected to cohesive failure. However, as shown in Fig. 3, the material of the invention can also be prepared to be capable of forming an image so that the whole of the heated thermosoftening colorant layer remains on the support by adjusting a composition of the thermosoftening colorant layer.

In the recording material shown in Fig.7, a release layer can be provided additionally on the outer surface of the thermosoftening colorant layer. If this release layer is provided, the attachment of thermosoftening material to the thermal head can be prevented when heat is drawn by the thermal head from the heat melting coloring layer side.

The release layer prevents the blocking phenomenon or sticking phenomenon.

The release layer is preferably formed by a conventional resin composition which can prevent the foregoing sticking phenomenon. For example, the composition, preferably, includes a resin composition containing (A) silicone type resin, (B) at least one selected from the group consisting of polyester resin, polyamide resin, cellulose type resin, acryl resin and fluorine containing resin and if necessary, (C) polyisocyanate compounds.

The silicone type resins may be represented by the following formula:
wherein R represents an organic group, k is an integer of not less than 1.

The resins preferably applicable include, for example, organopolysiloxane, modified polysiloxane resin, silicon modified acryl resin, silicon modified urethane resin, silicon modified urea resin, and silicone-modified epoxy resin. Such silicone modified resins are those prepared by modifying, for example, acryl resin, urethane resin, urea resin or epoxy resin by making use of polysiloxane.

In the above-mentioned various types of silicone-modified resins, the silicone contents thereof are within the range of, usually, 1 to 90% by weight and, preferably, 5 to 50% by weight.

These silicone resins may be used independently or in combination.

Among these silicone resins, the above-given various silicone-modified resins are preferably used.

Such silicone resins are preferable to be hardened with a cross-linking agent.

The cross-linking agent includes, without special limitation, an isocyanate, an aziridine, and an epoxy, for example.

The silicone resin content of a release layer is within the range of, normally, 1 to 100 wt% and, preferably, 10 to 80 wt%.

The silicone resins may be added in the form of a resin and they may also be contained uniformly in the hardened matter of a release layer. It is further allowed to contain them in the form of a fine powder into the release layer.

The polyamide resins include, without special limitation, Nylon 6, Nylon 8, Nylon 11, Nylon 66, and Nylon 610, for example. Besides the above, the copolymers thereof may also be used for.

The foregoing cellulose resins include, for example, those of cellulose esters such as acetyl cellulose, nitrocellulose, and acetylbutyl cellulose, cellulose ethers such as ethyl cellulose, methyl cellulose, benzyl cellulose, and carboxymethyl cellulose.

The foregoing acryl resins include, for example, the homopolymers of methyl acrylate, ethyl acrylate, methyl methacrylate, ethyl methacrylate, acrylonitrile, acrylamide, and the derivatives thereof, and copolymers of various kinds of acryl monomers with vinyl acetate, vinyl chloride, styrene, or anhydrous maleic acid.

The foregoing fluoro-containing resins include, for example, ethylene tetrafluoride resin, ethylene tetrafluoride-propylene hexafluoride copolymer resin, ethylene-tetrafluoride-perfluoroalkoxyethylene copolymer resin, ethylene trifluorochloride resin, ethylene tetrafluoride-ethylene copolymer, vinylidene fluoride resin, and vinyl fluoride resin.

Such fluoro-containing resins may be used independently or in combination.

The above-given various kinds of resins may be added in the form of a resin and they may also be contained uniformly in the hardened matter of a release layer. It is further allowed to contain them in the form of fine powder into the release layer.

The release layer is also allowed to contain, for example, inorganic or organic fine particles such as those of fluororesin, metal powder, or silica gel, a surfactant, and a lubricant.

Such release layers are further allowed to contain, besides the above-given components, additives such as a wax, a surfactant, a higher fatty acid derivative, a higher aliphatic alcohol, a higher aliphatic ether, and a phosphoric acid ester.

The compounding proportion of the components given above may suitably be determined to form such a release layer as described above.

The release layer is to be formed on the outermost layer of a heat-sensitive recording material, by adopting a coating method in which a solvent is used.

If the thickness of such release layer is not less than 0.01 µm, it would be good enough. However, it is practically within the range of 0.03 to 30 µm.

In the recording material shown in Fig. 7, when thermosoftening colorant layer 7 has either no or less self-supportability, it is allowed to provide the peelable support of which will be described later so as to assist the peelability. It is also allowed to give the above-mentioned release property to a peelable support. It is further allowed to provide the release layer onto the outer surface of either the peelable support 11 or support 6.

### 2. Modification example 1

The heat-sensitive recording material shown in Fig. 9 is a modification example of the heat-sensitive recording material shown in Fig. 7.

In heat-sensitive recording material 5a shown in Fig. 9, thermosoftening layer 9 and thermosoftening colorant layer 7 were laminated in this order on the surface of support 6.

The material of the above-described support is the same as that of the support of the heat-sensitive recording material shown in Fig. 7.

Thermosoftening layer 9 can be formed either by compounding the same binder as that used for forming the foregoing thermosoftening colorant layer, a an adhesive composition or a thermomelting material, and a resin having a relatively low softening point or having a low glass-transition point Tg, which is selected from the group consisting of, for example, ethylene copolymers such as an ethylene-vinyl acetate copolymer and an ethylene-ethyl acrylate copolymer; polyamide resins; polyester resins; polyurethane resins; acryl resins; and vinyl chloride resins; or, by using a conventionally known pressure-sensitive adhesive.

Such adhesives include, for example, a rosin adhesive; unmodified or modified rosin adhesives such as a hydrogenated rosin adhesive, a rosin maleic acid adhesive, a polymeric rosin adhesive, and a rosin phenol adhesive; a terpene adhesive; a petroleum resin adhesive; and the modified adhesives thereof.

The thermomelting materials applicable thereto include the same as those used in the foregoing thermosoftening colorant layer.

The thickness of the thermosoftening layer is within the range of, normally, 1 to 50 µm and, preferably, 1.5 to 10 µm.

Such thermosoftening layer is allowed to be colorless. If a ground-color is to be given to a recording image, it is preferable to contain, for example, a suitable colorant such as a white or light-colored pigment.

In heat-sensitive recording material 5a shown in Fig. 9, thermosoftening layer 9 and support 6 are in a tightly adhered state in advance. Therefore, when applying heat imagewise from the side of support 6, for example, by making use of a thermal head, for example, heat-applied thermosoftening colorant layer 7 and thermosoftening layer 9 are thereby mixedly fused so that the fixability of two layers may be enhanced. When thermosoftening colorant layer 7 is peeled off after heat was applied, at least a part 7a of the heat-applied thermosoftening colorant layer 7 remains on the thermosoftening layer 9, as shown in Fig. 10.

In heat-sensitive recording material 5a shown in Fig. 9, it is also allowed to provide a further release layer onto the outer surface of thermosoftening colorant layer 7. If this is the case and when applying heat from the thermosoftening colorant layer side through a thermal head, the adhesion of the colorant to the thermal head may be prevented.

In heat-sensitive recording material shown in Fig. 9, the thermosoftening colorant layer 7 is also allowed to contain, for example, a release agent such as silicone resin, polyester resin, polyamide resin, cellulose resin, acryl resin, or a polyisocyanate compound.

It is further allowed to provide a peelable support layer onto the thermosoftening colorant layer. i.e. onto the outer surface of the colorant layer. It is the matter of course that a release layer may be provided, if required, onto the peelable support layer.

Such peelable support layer is so provided as to assist the thermosoftening colorant layer to be peeled off when the thermosoftening colorant layer has either no or less self-supportability.

Such peelable support layer may be formed by using, without special limitation, a thermoplastic resin, provided, the resin has a mechanical strength as much as the layer can be peeled off. Among these resins, those having a relatively high glass transition temperature Tg, such as, polyacrylate resins, cellulose resins, polycarbonate resins and polyparabanic acid resin, may preferably be used.

In heat-sensitive recording material 5b shown in Fig. 11, peelable layer 10, thermosoftening layer 9, and thermosoftening colorant layer 7 are laminated in order on the surface of support 6. Similar to the recording material shown in Fig. 9, this recording material is allowed to have a peelable support layer 11 and a release layer, if required.

In this recording material, the support, thermosoftening layer, thermosoftening colorant layer, peelable support layer, and anti-sticking layer thereof are the same as those of the heat-sensitive recording materials shown in Fig. 7 and 9.

The peelable layer, which functions to smoothly peel a thermosoftening layer apart from a support, may be formed by compounding the same binder as that used for forming the above-described thermosoftening colorant layer or thermosoftening layer, and silicone resin. In this case, it is also allowed that a ground color may be given, if required, by adding a colorant.

The thickness of such a peelable layer is within the range of, normally, 0.1 to 10 µm and, preferably, 0.2 to 5 µm, so as not to hinder thermal response.

The peelable support layer described above is preferably provided on the colorant layer by a coating or laminating method. The coating method is more preferable, and the coating is carried out by using a solvent method or an emulsion method. The coating method includes te known techniques such as gravure-coater method, a wire-bar coating method, an air-knife coating method and a dip-coater method.

Also in the heat-sensitive recording material shown in Fig. 11, when heat is applied thereto from the side of support 6 or thermosoftening colorant layer 7 through a thermal head, for example, heat-applied thermosoftening colorant layer 7, thermosoftening layer 9, and peelable layer 10 are mixedly fused to enhance the fixability among the layers. On the other hand, in the unheated portions of peelable layer 10, the peelability of peeling apart from thermosoftening layer 9 is greater and, in the heat-applied portions thereof, thermosoftening layer 9 and peelable layer 10 tightly adhere to each other and, therefore, as shown in Fig. 12, heat-applied peelable layer 10, thermosoftening layer 9, and thermosoftening colorant layer 7 each remain on the surface of support 6 after a peeling operation was completed, and thereby an image is formed.

In this case, the peeling operation may be readily performed, because peelable support layer 11 is provided.

Further in heat sensitive recording material shown in Fig. 11, the recording material of the invention may be one which peelable layer 10 and thermosoftening layer 9 are arranged reversely. That is; thermosoftening layer 9 is provided onto the surface of support 6 and peelable layer 10 onto thermosoftening layer 9. In such a layer arrangement, thermosoftening layer 9 and peelable layer 10 are separated from each other at the interface therebetween after forming an image. Therefore, when thermosoftening layer 9 contains a colorant, the ground color can be given to an image as aforementioned.

In each of the above-given examples, the heat-applied adhesion of a layer to the support, or the adhesion of a layer to a thermosoftening layer provided onto the support, is produced by meltingly adhering to or making miscible with each other layer upon application of thermal fusion. It is also allowed to use other adhesion mechanism.

It is further allowed to form an image in such a mechanism that a latex, which is capable of displaying a layer-making function and contained in advance in a thermosoftening colorant layer, is so changed as to be a thin layer by applying heat, and the thermosoftening colorant layer is made adherent to a support by the resulting thin layer.

In the case of heat-sensitive recording material 5c, see Fig. 13, provided, onto the surface of support 6, with a lamination of specially structured thermosoftening colorant layer 7b containing a colorant in the mesh-like or stone wall-like matrix thereof, colorant 7c, see Fig 14, is oozed out of the specially structured thermosoftening colorant layer 7b by applying heat as shown in Fig. 13, and, when peeling the specially structured thermosoftening colorant layer 7b apart from support 6, the oozed out colorant 7c remains on the surface of support 6, so that an image is formed.

The material may be improved by the provision of a peelable layer, thermosoftening layer, peelable support layer, release layer, and anti-fogging layer. Such peelable layer, thermosoftening layer, peelable support layer, and release layer are similar to those used in the recording materials shown in Figs. 7, 9, 11, and 12.

The purpose of providing an anti-fogging layer is to prevent the recorded image surface from staining when forming thermosoftening colorant layer 7b on a printed record surface or in the course of storing the recorded image.

It is also allowed that such anti-fogging layer may or may not functions by itself as a peelable layer, and such anti-fogging layer may be formed by compounding, for example, a thermosoftening resin, a thermofusible material, a filler, and a lubricant such as silicone resin, fluororesin, and surfactant.

Such anti-fogging layer are so designed thin as not to hinder colorant 7c from permeating therethrough. The thickness of the anti-fogging layer is within the range of, normally, 0.1 to 3 µm and, preferably. 0.2 to 1.0 µm.

In the above-described embodiments having various modification examples, various types of layers may be formed by adopting any of the coating techniques such as a reverse-roll coater method, an extrusion-coater method, a gravure-coater method, and a wire-bar coating method.

Embodiment 1 and the modification examples thereof are collectively shown in Fig. 15.

### -The second embodiment-

A heat-sensitive recording material, that is the preferable embodiment 2 of the invention, comprises a lamination of a mordant layer serving as the above-described image-receiving layer and a dye-supplying layer serving as the above-described colorant containing layer.

### 1. Basic constitution

The second embodiment is basically constituted by that, as shown in Fig. 16, a dye-supplying layer 15 containing a dye 14 and a mordant layer 16 are provided, through which, dye 14 of dye-supplying layer 15 is diffusively moved into the mordant layer 16 by applying heat energy from the side of the dye-supplying layer 15 or mordant layer 16 so that an image may be formed on the mordant layer 16 by the diffused dye 14, and the image-recorded mordant layer 16 is then separated from the dye-supplying layer 15. The separated mordant layer having the image thereon is used as an image recorded member by itself. The resulting image-recorded member functions as if it were, for example, an image-printed or image-drawn sheet of paper. Therefore, the mordant layer itself has no stickiness.

The dye-supplying layer contains a dye and a binder. In the dye-supplying layer, the dye thermally diffuses when heat energy is applied imagewise.

There is no special limitation to the dyes, provided that they may be diffused by heat, changed to be thermally diffusible, sublimable, vaporized, or thermally fusible.

In the meantime, the diffusibility of dye molecules is changed depending on the molecular weight thereof. Therefore, the molecular weight of the dye suitable for the invention is within the range of, normally, 50 to 4,000 and preferably, 100 to 1,000.

When the molecular weight of the dye is within the range of 100 to 1,000, the diffusibility of the dye becomes particularly preferable.

In this embodiment, the dye is diffusively moved into the mordant layer by applying heat. It is, therefore, preferable that the dye may readily be fused, sublimated, or vaporized by applying heat energy supplied from a thermal head.

The melting points, sublimating temperatures, or vaporizing temperatures each required for dyes are varied depending on what kind of recording apparatuses should be loaded with the above-mentioned heat-sensitive recording material and how to make a heat-sensitive record. Therefore, such preferable temperatures cannot absolutely be fixed. When using this type of heat-sensitive recording material with a facsimile communication apparatus, for example, the melting point, sublimating temperature, or vaporizing temperature for such dyes is within the range of, preferably, 60 to 300°C and, more preferably, 100 to 250°C.

Such dyes may be made present in the dispersed, dissolved, or molecular-dispersed state in the binder of which will be described later.

Such dyes include, for example, leuco dyes, i.e., soluble vat dyes, direct dyes, acid dyes, basic dyes, acid mordant dyes, metal complex dyes, sulfur dyes, vat dyes, azo dyes, disperse dyes, reactive dyes, oxidation dyes, and oil dyes.

In the invention, the above-given dyes may be used independently or in combination.

When two or more kinds of such dyes are used in combination and they are different from each other in tone, molecular weight, melting point, sublimating temperature, vaporizing temperature, and, therefore, in dispersion property, the tones and color density of an image can be controlled by suitably applying heat energy. For example, images such as multicolored or various color-density characters, drawings and marks may be formed on a mordant layer by applying suitable heat energy from an exothermic element.

The dye content of the whole dye-supplying layer is within the range of, normally, 5 to 80 wt% and, preferably, 10 to 50 wt%.

The amount of the dye to 100 parts by weight of the binder used is within the range of, normally, 5 to 300 parts by weight and, preferably, 10 to 200 parts by weight.

There is no special limitation to the above-described binders, provided that, when no heat is applied, they may be able to maintain such dyes stably, and that, when heat is applied, they may be softened or melted in themselves so as to make the dye movement ready.

Such binders include, for example, a thermoplastic resin, a thermofusible material, and a plasticizer.

The thermoplastic resins are similar to those having been described in the foregoing first embodiment.

In this invention, various kinds of the thermoplastic resins may be used independently or in combination. Among these thermoplastic resins, if a thermoplastic resin itself may be formed into a film or sheet shape, it functions not only as a binder but also as a support. Therefore, when such a thermoplastic resin capable of being formed in itself in a film or sheet shape is served as a binder, the resulting dye-supplying layer has a self-supportability to become self-supportable dye-supplying layer 15', as shown in Fig. 17, so that no support is required, and dye-supplying layer 15 and mordant layer 16 may readily be separated from each other.

The above-mentioned thermofusible materials are similar to those described in the foregoing first embodiment.

In this invention, various thermofusible materials may be used independently or in combination.

The plasticizers applicable to the invention may be selected, for example, from the group consisting of those of phthalic acid esters, phosphoric acid esters, adipic acid esters, sebacic acid esters, azelaic acid esters, citric acid esters, glycolic acid esters, trimellitic acid esters, phthalic acid isomer esters, polyesters, and epoxides.

The other plasticizers, besides the above, include, for example, those of fatty acid esters, fatty acids, silicone-oil, modified silicone-oil, fluorine-oil, and liquid paraffin.

The content of the above-described binders in the dye-supplying layer is within the range of, normally, 1 to 50 wt% and, preferably, 3 to 30 wt%.

If required, such dye-supplying layer is allowed to contain a thermal-dispersion aid, a filler, a pigment, an antioxidant, and UV-absorber.

The layer thickness of such dye-supplying layer is within the range of, normally, 0.5 to 30 µm and, preferably, 1 to 10 µm.

### 2. The first modification example

This dye-supplying layer may be either of the single-layered or of the multiple-layered as shown in Fig. 18.

In Fig. 18, dye-supplying layer 15 comprises three component layers, namely, a green dye-supplying component layer 15a supplying green dye, a red dye-supplying component layer 15b supplying red dye, and a yellow dye-supplying component layer 15c supplying yellow dye. The thicknesses of these three dye-supplying component layers, 15a, 15b, and 15c, may not necessarily be made the same with each other, but may suitably be made different from each other so as to meet the kinds of such dyes, because the diffusion distance of such dyes may be considered to be the thicknesses of the dye-supplying layer.

In the case where dye-supplying layer 15 comprises the above-described three component layers, the color dyes are moved to a mordant layer according to the heat energy applied, respectively, so that a recorded member having a colored image thereon may be obtained.

Each of the three component layers constituting the above-described dye-supplying layer is allowed not only to be compounded with different tone dyes as described above, but also to contain the dyes having a different molecular weight, melting point, or sublimating temperature, respectively.

The three component layers of the dye-supplying layer may be of the self-supportable type, as described above.

The mordant layer is a layer capable of forming an image thereon when it receives a dye being diffusively moved thereinto so as to be fixed by applying heat. When the dye diffuses to the mordant layer, the dye is fixed either in the binder of the mordant layer or on the surface of the mordant layer.

The materials for forming the mordant layer include, for example, thermoplastic resins, thermofusible materials, and plasticizers, each of which is similar to the binders normally used in the foregoing dye-supplying layer.

The thermoplastic resins, thermofusible materials, and plasticizers are exemplified in the foregoing description, and a further detailed exemplification will be omitted here. In the mordant layer, however, dyes are desired to have a higher solubility or miscibility than in the dye-supplying layer.

The thermoplastic resins preferably applicable to the invention include, for example, polyester resins, vinyl chloride resins, vinylidene chloride resins, and urethane resins.

Among the thermoplastic resins, some of the resins can function not only as a mordant layer capable of receiving a dye, but also as a support, provided, such resins itself can be formed into the film or sheet shape.

Therefore, as shown in Fig. 19, when mordant layer 16' is formed of a thermoplastic resin which can be formed into a film or sheet shape, such mordant layer can be self-supportable or can become a self-supporting mordant layer 16'. Therefore, a support is not necessary, and the dye-supplying layer 15 and mordant layer 16' can readily be separated from each other. It is also possible to make both dye-supplying layer and mordant layer self-supportable.

Such mordant layer can be formed with at least one selected from the group consisting of the above-given thermoplastic resins, thermofusible materials, and plasticizers. The mordant layer is further allowed to contain a chelating agent, an antioxidant, a UV-absorber, and a filler.

The fillers include, for example, silica, talc, calcium carbonate, alumina, acid clay, clay, magnesium carbonate, tin oxide, titanium white, graphite, setting resin particles, silicone resin particles, fluororesin particles, melamine resin particles, urea resin particles, benzoguanamine resin particles, acryl resin particles, styrene resin particles, boron nitride, copper, iron, aluminium, iron oxide, aluminium oxide, magnesium oxide, and titanium nitride. Besides the above-given fillers, there includes a colored filler. When compounding such colored filler into a mordant layer, the layer is ground-colored.

The mordant layer may be either colorless and transparent or ground-colored as mentioned above.

When the mordant layer is ground-colored, an image formed of a dye having a different color from the ground color may be distinctly displayed.

The mordant layer may be formed on a support either directly or with the interposition of an interlayer.

If such mordant layer itself has no self-supportability, the mordant layer may be formed; on the support directly or with the interposition of the sublayer of which will be described later; or on a dye-supplying layer directly or with the interposition of an interlayer; by adopting a coating method such as a hot-melt coating method, an aqueous coating method, or a coating method in which an organic solvent is used; or by laminating it on. If such mordant layer has a self-supportability, it may be formed in the film or sheet shape in a extrusion moulding process.

### 3. The second modification example

In this modification example of the second embodiment suitable for the invention, the heat-sensitive recording material comprises, as shown in Fig. 20, support 6 provided either to mordant layer 16 on the side opposite to dye-supplying layer 15 or to dye-supplying layer 15 on the side opposite to mordant layer 16; or, the recording material is comprised of one each of support 6 provided to both sides of mordant layer 16 and dye-supplying layer 15; so as to smooth the separation of mordant layer 16 from dye-supplying layer 15.

In this modification example, a support should be provided, because the self-supportability of the dye-supplying layer and/or the mordant layer each have not satisfactory mechanical strength for separating these layers from each other.

Such support is desired to have excellent heat resistance and dimensional stability. The materials for such support are as given before.

The support is also allowed to contain a colorant. When the support contains a colorant and the support and a mordant layer are directly adjacent to each other, the color of the support colored by the colorant will become the ground color to an image formed on the mordant layer so that the contrast of the image may be distinct.

In the second embodiment of the invention, the heat-sensitive material basically has a dye-supplying layer, a mordant layer and, if required, a support, as aforedescribed. On the other hand, in the layer arrangement of the heat-sensitive recording material, it is allowed to form a release layer 13; on the surface of dye-supplying layer 15 and/or mordant layer 16 which is the outermost layer, as shown in Fig. 21; on self-supportable dye-supplying layer 15' and/or self-supportable mordant layer 16' each of which is the outermost layer, as shown in Fig. 22(a) and 22(b); or, on the surface of support 6, as shown in Fig. 23.

In the above-described cases, the release layer has the same functions or performance and may also be formed of the same compositions as those described in the foregoing first embodiment,

In the case of a heat-sensitive recording material having a mordant layer formed on a support, an adhesive sublayer 17 may be interposed between support 6 and mordant layer 16 with the purposes of enhancing the adhesion of mordant layer 16 and support 6 to each other and producing a ground color to an image formed on mordant layer 16, as shown in Fig. 24.

When such an adhesive sublayer for producing a ground color is provided, the contrast of the dye-image formed on mordant layer 16 can be made distinct.

For example, such an adhesive sublayer as described above may be formed by using a mixture of a known composition serving as an adhesive and a colorant.

The kinds of such adhesives are as aforedescribed.

The above-described colorants include, for example, inorganic and organic pigments.

Such inorganic pigments as described above include, for example, titanium oxide, carbon black, zinc oxide, Prussian blue, cadmium sulfide, iron oxide, and the chromates of lead, zinc, barium or calcium.

Such organic pigments as described above include, for example, those of the azo, thioindigo, anthraquinone, anthanthrone, and triphenyloxazine types, phthalocyanine pigments such as copper phthalocyanine and the derivatives thereof, and a quinacridone pigment.

The thickness of such an adhesive sublayer is within the range of, normally, 0.3 to 3 µm and, preferably, 0.5 to 2 µm.

As shown in Fig. 25, it is also allowed to interpose a peelable layer 10 between mordant layer 16 and dye-supplying layer 15, or between a self-supporting type mordant layer and a self-supporting type dye-supplying layer, because the interpostion of the peelable layer makes it smooth and easy to separate those two layers when it is interposed.

As shown in Fig. 26, it is further recommended to interpose anti-fogging layer 21 between mordant layer 16 and dye-supplying layer 15, or between a self-supporting type mordant layer and a self-supporting type dye-supplying layer. If the anti-fogging layer 21 is interposed, the mordant layer or the self-supporting type mordant
layer can effectively be prevented from stains produced by the natural diffusion of dyes which may occur when forming the mordant layer on the dye-supplying layer or the self-supporting type dye-supplying layer, or when the resulting heat-sensitive material is stored for a long time.

The peelable layer and anti-fogging layer may be prepared by compounding, for example, a thermosoftening resin, a heat-melting substance, a filler, a lubricant, a release agent such as silicone resin, fluororesin, and surfactant.

The thicknesses of both the peelable layer and the anti-fogging layer are within the range of, normally, 0.3 to 3 µm and, preferably, 0.5 to 2 µm, and, the thinner, the better.

The above-described interlayer is also allowed to have a dual-layered structure in which one layer is arranged to be the peelable layer and the other layer to be the anti-fogging layer, or to have the functions of the peelable and the anti-fogging layers.

Such heat-sensitive materials thus prepared can be used in the tape, sheet or the like form.

According to the heat-sensitive materials in the second and third embodiments, an image can be formed, for example, in the following manner.

By making use of a thermal head, heat pulses are applied to the heat-sensitive material from the side of the surface capable of being heated, and thereby the dye-supplying layer or the self-supporting type dye-supplying layer and the mordant layer or the self-supporting type mordant layer are heated locally corresponding to a desired original print or transferring pattern.

When the dye-supplying layer and the mordant layer are imagewise heated, the dyes contained in the dye-supplying layer diffuse into the mordant layer, so that an image is formed on the mordant layer. Then, when the dye-supplying layer is separated from the mordant layer, a recording medium having the image on the mordant layer is obtained. The recording medium itself may be handled as if it were a paper on which the image was drawn. Therefore, the mordant layer itself has no stickiness.

Fig. 27 collectively illustrates both of the second embodiment and the modification example thereof.

### - The third embodiment -

The heat-sensitive recording materials each relating to the third embodiment comprise a dye-supplying layer as a colorant layer, and either a sticky mordant layer or a mordant layer having an adhesive layer on its side facing the dye-supplying layer; or, they comprise each a mordant layer as an image-receiving layer, and either an adhesive dye-supplying layer or a dye-supplying layer having an adhesive layer on the side facing the mordant layer, as the colorant layer.

The third embodiment of the heat-sensitive recording material is based on the following principle:
(a) From a layer having contained in advance a heat-diffusible dye to the other layer, the dye is to be diffusively transferred by heat;
(b) The recipient layer of the dye transferred thereto by the heat-diffusion is to be separated from the other layer; and
(c) The recipient layer of the dye, or the layer having contained in advance a heat-diffusible dye, is to be made adhesive.

The heat-sensitive recording materials of the third embodiment based on the above-described principle can be modified variously.

### 1. The first Modification example

As shown in Fig. 28, this modified heat-sensitive recording material is a laminate comprising an adhesive mordant layer 18b serving as both as an adhesive layer and a mordant layer, and dye-supplying layer 19a containing a heat-diffusible dye, each laminated together. The laminate is so prepared as to enable separation of the adhesive mordant layer 18b from the dye-supplying layer 19a.

The components, compositions and layer arrangements of the dye-supplying layer are the same as those of the dye-supplying layer described in the foregoing second embodiment.

The adhesive mordant layer can be prepared by adding an adhesive composition to the components of the mordant layer described in the foregoing second embodiment.

There is no special limitation to the adhesive compositions, but any one for general use may be used.

The typical examples of such adhesive compositions include, for example; natural rubber; those of the chloroprene, butyl rubber, polyacrylic acid ester, nitrile rubber, polysulfide, and silicone rubber types; and those prepared with reclaimed rubber, SBR, polyisoprene, polybutyl ether, and Buna-N.

Among the above-given examples, more preferable ones are natural rubber, chloroprene rubber, butyl rubber, and polyacrylates.

Such adhesive compositions are further allowed to contain suitably a tackifier, a plasticizer, a filler, an anti-ageing agent.

The tackifiers include, for example, polyterpene resin, gum rosin, rosin derivatives, oil-soluble phenol resin, cumarone indene resin, cumarone resin, indene resin, and petroleum hydrocarbon resin.

The plasticizers include, for example, mineral oil, liquefied polybutene liquid polyacrylate, and lanolin.

The fillers include, for example, zinc white, hydrate aluminium, titanium oxide, calcium carbonate, clay, pigment, silica, and aluminium hydroxide.

The anti-ageing agents include, for example, di-thiocarbamate, a metal chelating agent, and antioxidant.

The content of the adhesive composition in a sticky mordant layer may not always be fixedly determined, because it depends on the kinds of the components of the adhesive mordant layer and the content thereof. To sum up, the content thereof may be suitably determined so that an adhesive mordant layer may easily be peeled off from a dye-supplying layer, and that the adhesive composition may be able to display an adhesive strength of the order that the adhesive mordant layer may easily be pasted up on the other member. Normally, the content of the adhesive composition of the adhesive mordant layer is within the range of 1 to 90 wt%.

In the heat-sensitive recording material of the first modification example, when applying heat energy from the dye-supplying layer side or the adhesive mordant layer side, dyes are diffusively transferred from the dye-supplying layer into the adhesive mordant layer and an image is then formed on the adhesive mordant layer. When the adhesive mordant layer is separated from the dye-supplying layer, the adhesive mordant layer having an image formed thereon can be obtained, because the dye-supplying layer and the adhesive mordant layer are so laminated as to be separated from each other. The adhesive mordant layer having the image formed thereon is handled as an independent recorded medium having the image formed thereon. The image formed on the recorded medium is excellent in image storage stability, because it is formed on the independent recorded medium.

The image-formed mordant layer can be pasted up as a label on other articles.

Further, if an adhesive mordant layer is separated from a dye-supplying layer and is then pasted up on another dye-supplying layer separately prepared, another new heat-sensitive recording material can be prepared. If the new material is applied with heat energy again, another image can be superposed on the sticky mordant layer having the image formed thereon. If the kind of the dye contained in the dye-supplying layer separately prepared is different from that contained in the dye-supplying layer used before separating the adhesive mordant layer, the images each formed superpositively on the adhesive mordant layer may be multicolored or may have the different color tones.

### 2. The second modification example

As shown in Fig. 29, this modified heat-sensitive recording material is a laminate comprising; non-adhesive mordant layer 18a which forms an image upon receipt of a dye being diffusively transferred thereto; dye-supplying layer 19a which contains a dye being diffusively transferred by applying heat energy; adhesive layer 20 which is interposed between layer 18a and layer 19a; and adhesive layer-attached mordant layer 18b which can be separated from dye-supplying layer 19a; each of which are laminated.

The non-adhesive mordant layer and the dye-supplying layer are the same as the mordant layer described in the foregoing second embodiment.

Such adhesive layer is arranged when both of the mordant layer and the dye-supplying layer are either non-adhesive or only slightly adhesive.

The adhesive layer is prepared so as to adhere to a dye-supplying layer, whereby, as shown in Fig. 29, the adhesive layer attached to mordant layer 18b can be separated from dye-supplying layer 19a.

An adhesive layer can be separated from a dye-supplying layer, but not from a mordant layer, by suitably adjusting the compositions of the adhesive layer components, taking the compositions of the dye-supplying layer and the mordant layer into consideration. As will be described later, if a peeling layer is interposed between the adhesive layer and a layer which may be separated from the adhesive layer, an adhesive layer attached-mordant layer can readily be separated.

In either way, the above-described adhesive layer can be prepared of a tackifier which is the same as those for the aforedescribed adhesive mordant layer.

The thickness of such an adhesive layer described above is within the range of, usually, 0.3 to 500 µm and, preferably, 0.5 to 50 µm.

In the heat-sensitive recording material shown in Fig. 29, an image is formed on the mordant layer by applying heat energy, and the mordant layer having the image formed thereon is separated from a dye-supplying layer. To be more accurate, in the heat-sensitive material, the mordant layer united with an adhesive layer in a body is separated from the dye-supplying layer.

The mordant layer thus separated and made independent still has an adhesive layer, therefore, the adhesive layer-attached mordant layer has the equal or similar functions to those of the adhesive mordant layer of the first modification example, so that it may be handled as a label and may be utilized as a mordant layer having thereon a multicolored or different color-tone image.

### 3. The third modification example

The heat-sensitive recording material of Modification Example 3 is a laminate comprising; a dye-supplying layer containing a dye which is diffusively transferred by applying heat energy; an adhesive layer; and a mordant layer forming an image upon receipt to the dye diffusively transferred from the dye-supplying layer; wherein the layers are laminated in the above order, and the mordant layer and the adhesive layer-attached dye-supplying layer can be separated apart.

To be more concrete, in the heat-sensitive recording material, as shown in Fig. 30 each of the layers are laminated so that the adhesive layer 20 may be interposed between non-adhesive mordant layer 18a and dye-supplying layer 19a, and mordant layer 18a and the adhesive layer-attached dye-supplying layer 19b may be separated apart.

While the adhesive layer may be peeled apart from the mordant layer, it still adheres to the dye-supplying layer. Such adhesion thereof may be obtained by controlling each component of the tackifier so as to meet the compositions of the mordant layer and dye-supplying layer.

The thickness of the adhesive layer is as same as that in the second modification example.

As is same as in the first and second modification examples, in this example also, an image may be formed on a mordant layer by applying heat energy, and the mordant layer having the image thereon may be separated from an adhesive layer-having dye-supplying layer.

Similar to the case of the first modification example, this mordant layer is handled as an independent image-recorded medium. The image formed on the recorded medium is excellent in image-storage stability, because the image is formed on the independent medium.

When a separate and independent mordant layer having an image thereon is attached to another separately prepared and adhesive layer attached dye-supplying layer, a further new heat-sensitive recording material can be prepared. When applying heat energy again to the newly prepared heat-sensitive recording material, another image can be superposed upon the mordant layer having the image thereon. If the dye of this separately prepared adhesive layer attached dye-supplying layer is made different from the dye of the sticky layer attached dye-supplying layer which did not yet separate the mordant layer therefrom, the image superposed on the mordant layer can be multicolored or made it to have the other tone than the original tone.

### 4. The fourth modification example

The heat-sensitive recording material of this modification example comprises an adhesive dye-supplying layer containing a dye diffusively moved by applying heat energy thereto, and a mordant layer forming an image thereon upon receipt of the dye diffusively moved thereto so that the sticky dye-supplying layer and the mordant layer can be separated from each other.

To be more concrete, such heat-sensitive recording materials include, as shown in Fig. 31, a laminated member comprising non-adhesive mordant layer 18a and adhesive dye-supplying layer 19b which also serves as an adhesive layer and contains a thermodiffusible dye.

Such mordant layer as described above is similar to that detailed in the foregoing second embodiment.

Such an adhesive dye-supplying layer can be prepared by adding an adhesive to the composition of preparing the dye-supplying layer detailed in the foregoing second embodiment. Of the adhesives, the description has already been made in the foregoing first modification example.

In the heat-sensitive recording material of this fourth modification example, the adhesive dye-supplying layer thereof can function as same as that of the aforedescribed adhesive layer attached dye-supplying layer, and displays the same or equivalent functional effects as in the third modification example.

### 5. Layer arrangement

The heat-sensitive recording material relating to the third embodiment basically comprises, as shown in the foregoing first to fourth modification examples, an adhesive mordant layer and a dye-supplying layer, an adhesive layer attached mordant layer and a dye-supplying layer, a mordant layer and an adhesive layer attached dye-supplying layer, or a mordant layer and an adhesive dye-supplying layer.

In such a layer arrangement as mentioned above, the dye-supplying layer is not limitative to have a single-layer arrangement, but is allowed to have a plurality of layers such as a three-layer arrangement. -Refer to Fig. 32.-

In Fig. 32, dye-supplying layer 19 comprises, for example, the following three component layers, namely, green dye-supplying layer 19A containing green dyes, a red dye-supplying layer 19B containing red dyes, and yellow dye-supplying layer 19C containing yellow dyes. The thicknesses of these three dye-supplying layers may not necessarily be the same, but may be so variable appropriately to meet the kinds of the dyes.

In the case of such three-layered dye-supplying layer, each color-forming dye moves into the mordant layer according to heat energy applied, so that a recording medium having a color-image thereon can be obtained.

Each component layer of such three-layered dye-suppling layer is allowed not only to be compounded with dyes each different in tone as described above, but also to contain the dyes each different in molecular weight, melting point or sublimating temperature.

Such three-layered dye-supplying layer may be of self-supportable, or, among the three component layers, at least one on the mordant layer side may have a stickiness.

In the above-described basic constitution, the dye-supplying layer and mordant layer are so made self-supportable as to readily peel apart the dye-supplying layer from the mordant layer. To make the dye-supplying layer and mordant layer self-supportable, each of the layers is preferable to use therein a binder capable of forming the recording material into the film or sheet shape.

When the dye-supplying layer and mordant layer are not self-supportable, it is preferable to provide a support.

To be more concrete, as shown in Fig. 33, it is preferable to provide the support to dye-supplying layer 19a or adhesive dye-supplying layer 19b on the side thereof opposite to adhesive mordant layer 18b or mordant layer 18a. When laminating the support onto the dye-supplying layer or the adhesive dye-supplying layer, the mechanical strength of the dye-supplying layer or the adhesive dye-supplying layer may be enhanced, as well as the adhesive mordant layer or the mordant layer may smoothly be peeled apart from the adhesive dye-supplying layer or the dye-supplying layer.

According to the material of the invention, a transparent support is preferably provided on the outer surface of the image receiving layer.

As shown in Fig. 34, it is preferable to provide transparent support 6a onto mordant layer 18a or adhesive mordant layer 18b on the side thereof opposite to adhesive dye-supplying layer 19b or dye-supplying layer 19a. When providing the transparent support, not only the same effects as those of the above-described support can be displayed, but also the surface of the image-formed mordant layer can be protected when the separated mordant layer is so pasted as to serve as a label over the other material or article.

In other words, when the above-described transparent support is provided to the above-described mordant layer on the side thereof opposite to the dye-supplying layer, or it is provided to the adhesive mordant layer on the side thereof opposite to the dye-supplying layer, not only the mordant layer or the adhesive mordant layer can readily be separated, but also the image formed on the mordant layer or the adhesive mordant layer can be prevented from being scratched or rubbed, because the transparent support is provided onto the surface of the mordant layer or the adhesive mordant layer pasted over the other article, and such transparent support can serve as a surface protective layer.

It is also preferable to provide a transparent support onto the surface of a mordant layer or an adhesive mordant layer and, at the same time, to provide a support onto the surface of an adhesive dye-supplying layer or a dye-supplying layer.

In either way, it is preferable that such support including the transparent support should have excellent heat resistance and dimensional stability.

The composing materials of such supports are the same as those described in the foregoing first embodiment of the invention.

A support having a clearness may be used as the transparent support. The wording, 'clearness' herein means a transparency of the order that an image on a mordant layer can at least be recognized.

The thicknesses of such supports including the above-described transparent support are not specially limitative, but any thicknesses may be selcted. However, the thickness thereof is, normally, not thicker than 30 µm and, preferably, within the range of 2 to 30 µm.

For example, it is also preferable to interpose a peelable layer 10 (not shown); between the adhesive mordant layer 18b and dye-supplying layer 19a, as shown in Fig. 28; between the adhesive layer 20 and dye-supplying layer 19a, as shown in Fig. 29; between the adhesive layer 20 and mordant layer 18a, as shown in Fig. 30; or between mordant layer 18a and the adhesive dye-supplying layer 19b, as shown in Fig. 31.

When the above-described peelable layer is provided, the peeling force of a mordant layer or an adhesive mordant layer from an adhesive dye-supplying layer or a dye-supplying layer and vice versa may be so adjusted as to improve the peelability.

The above-described peelable layer is similar to those described in the foregoing first embodiment of the invention. For example, such a peelable layer may be formed of silicone resin, silicone-modified resin, wax, or a surfactant.

The thickness of the peelable layer is within the range of, normally, 0.1 to 10 µm and, preferably, 0.2 to 5 µm.

In the heat-sensitive recording material, it is preferable to interpose anti-fogging layer 21 as an interlayer between mordant layer 18a or adhesive mordant layer 18b and adhesive dye-supplying layer 19b or dye-supplying layer 19a, as shown in Fig. 35. In Fig. 35, numeral 10 indicates a peelable layer.

When the above-described anti-fogging layer is interposed between the mordant layer and the dye-supplying layer, it can effectively prevent the mordant layer or the adhesive mordant layer from being stained by the natural diffusion of dyes caused either when forming the mordant layer or the adhesive mordant layer on the adhesive dye-supplying layer or the dye-supplying layer, or when the heat-sensitive recording material is being stored for a long time.

The above-described anti-fogging layer may usually be formed of the same binder as that used in the dye-supplying layer and an anti-foggant.

The anti-foggant may be prepared by making use of the aforedescribed thermoplastic resin, thermofusible material, and filler.

The thickness of the anti-fogging layer is within the range of, normally, 0.3 to 10 µm and, preferably, 0.5 to 5 µm.

When such an anti-fogging layer is interposed between a peelable layer and a dye-supplying layer, or between a mordant layer and a peelable layer, it can effectively prevent the mordant layer from the fogging phenomenon produced by the dyes moving from the dye-supplying layer in the course of manufacturing or coating a heat-sensitive recording material or during the storage of the recording material.

When trying to simplify the layer arrangement so as to eliminate the complication of providing a special anti-fogging layer, it is preferable to compound the anti-foggant into the peelable layer.

When the peelable layer contains the antifoggant, it can effectively prevent the mordant layer from a fogging phenomenon produced by the dyes moved from the dye-supplying layer in the course of manufacturing or coating the heat-sensitive recording material, or during the storage thereof.

In the heat-sensitive recording material, it is preferable to form a non-adhesive release layer on the outer surface of at least one of the outermost layers of the layer arrangement.

However the release layer 13 may be formed on the surface of support 6 and/or a transparent support.

When the mordant layer or adhesive mordant layer contains a non-diffusible colorant, or when arranging a non-diffusible colorant layer containing a non-diffusible colorant onto the surface of the dye-supplying layer or the adhesive dye-supplying layer, the mordant layer or the adhesive mordant layer is provided with ground-color by the above-mentioned non-diffusible colorant, so that a higher contrast may be produced between the ground-color and an image formed by the dyes moved from the dye-supplying layer or the adhesive dye-supplying layer. Therefore, the resulting image can be displayed more sharper and clearer.

### 6. Application of the heat-sensitive recording material

The heat-sensitive recording material thus prepared may be used in the form of tapes or sheets, for example.

When using such a heat-sensitive recording material as mentioned above, an image may be formed in the following manner, for example:

Heat pulses are applied by using a thermal head to the heat-sensitive recording maerial from the heat-applicable side thereof so as to heat locally a dye-supplying layer or an adhesive dye-supplying layer and an adhesive mordant layer or a mordant layer each corresponding to a desired printed character of pattern which is to be transferred.

The temperatures of the locally heated portions of the dye-supplying layer or adhesive dye-supplying layer and the adhesive mordant layer or mordant layer are raised so that the locally heated portions thereof are rapidly melted, and the dyes contained in the dye-supplying laye or adhesive dye-supplying layer are thereby diffusively moved to the adhesive mordant layer or mordant layer so as to form the image on the adhesive mordant layer or mordant layer. When separating the dye-supplying layer or adhesive dye-supplying layer and the adhesive mordant layer or mordant layer from each other, a medium having the image recorded on the adhesive mordant layer or mordant layer thereof can be obtained.

In the case that the image-recorded medium obtained above is an adhesive mordant layer or an adhesive layer attached mordant layer, the medium can also serve as a label when it is pasted upon the surface of other material or article.

In the meantime, the above-described recorded medium having the image is superposed on the other separately prepared dye-supplying layer having contained in advance other dyes of the different kind or tone from those of the dye having been contained in the dye-supplying layer used first.

As in the preceding procedures, heat pulses are applied by a thermal head to this newly prepared heat-sensitive recording material from the heat-applicable side thereof, and the newly formed image may be superposed on the adhesive mordant layer or adhesive layer attached mordant layer having already had the image thereon. The above-described procedures may be repeated many times.

Upon completion of the procedures, a recording material having a multicolored or different tone image on the adhesive mordant layer or the sticky-layer attached mordant layer can be prepared. The resulting recording material can also serve as a label, as described above.

As shown in Fig. 31, in the case that the heat-sensitive recording material is a laminate member comprising an adhesive dye-supplying layer 19b and mordant layer 18a each laminated together, heat energy is applied to the mordant layer so as to form a certain image thereon and the mordant layer is then peeled apart from the recording material. The mordant layer thus peeled apart is then superposed on the other separately prepared adhesive dye-supplying layer having contained in advance the dyes of the different kind or tone from those of the dyes contained in the adhesive dye-supplying layer used first.

As in the preceding procedures, heat pulses are applied by a thermal head to this newly prepared heat-sensitive recording material from the heat-applicable side thereof, and the newly formed image may be superposed on the mordant layer having already had the image thereon. The above-described procedures may be repeated many times.

Upon completion of the procedures, a mordant layer having a multicolored or different tone image thereon can be prepared. The resulting mordant layer can serve as an independent recording medium, as described above.

Fig. 36 collectively illustrates both of the third embodiment of the invention and the embodiment of the modification example thereof.

### EXAMPLES

The invention will be further detailed with reference to the following examples.

### Example 1

### 1. Formation of a thermosoftening layer

A coating solution prepared by dispersing the following thermosoftening layer compositions into water was coated onto a smooth-surfaced paper sheet having a Beck's surface-smoothness of 200 seconds, and the resulting layer was dried up so as to complete a thermosoftening layer. The thickness of the layer is 10 g/m².

### Compositions of the thermosoftening layer

| | |
|---|---|
| Paraffin wax | 20 wt% |
| Polyester polymer, (having a weight-average molecular weight Mw = 20,000) | 40 wt% |
| Titanium oxide | 40 wt% |

### 2. Formation of a thermosoftening colorant layer

A coating solution containing the following thermosoftening colorant layer compositions was coated in an amount of 3 g/m² onto the thermosoftening layer prepared in the manner described in the preceding paragraph 1, so that a thermosoftening colorant layer was formed.

### Compositions of thermosoftening colorant layer

| | |
|---|---|
| Paraffin wax emulsion (as the solids) | 60 wt% |
| A dispersion of carbon black/water | 20 wt% |
| Acryl latex | 20 wt% |

### 3. Formation of release layer

A coating solution containing the following release layer compositions was coated in a thickness of 6 g/m² onto the thermosoftening layer prepared in the manner described in the preceding paragraph 2, so that a release layer was formed.

### Compositions of release layer

| | |
|---|---|
| Acryl latex | 8 wt parts |
| A dispersion of urethane/silicone/water | 1 wt part |
| A dispersion of aromatic polyester polymer/water | 1 wt part |

### 4. Formation of image

By making use of a thermal printer loaded with a 260 mm width line-head, and having an applicable energy capacity of 25 mj/mm² and a pressure capacity of 7 kg/head, a heat-energy was applied, from the release layer side, to the heat-sensitive recording material prepared in the processes described in the preceding paragraphs 1 through 3, so that an image was formed.

As the results thereof, the thermosoftening layer and the thermosoftening colorant layer were peeled off from each other, so as to obtain an image formed by the thermosoftening colorant layer remaining imagewise on the thermosoftening layer.

The thermosoftening layer and the thermosoftening colorant layer were peeled off at an angle of 60°.

### Example 2

A heat-sensitive recording material was prepared in the same manner as in Example 1, except that a peelable layer was so formed as to have a coated thickness of 0.5 µm, between a thermosoftening layer and a thermosoftening colorant layer, by coating the following composition:

### Peelable layer composition

| | |
|---|---|
| Paraffin wax | 80 wt% |
| Polyoxyethylene stearyl ether | 20 wt% |

When an image was formed by applying heat energy from the release layer side in the same manner as in Example 1-(4), the thermosoftening layer and the thermosoftening colorant layer were readily peeled apart from between the interface thereof, and the peelable layer and the thermosoftening colorant layer were mixedly fused imagewise on the thermosoftening layer so that an image was produced.

### Example 3

A heat-sensitive recording material was prepared in the same manner as in Example 1, except that a peelable support layer containing 100% of polycarbonate resin was so formed as to have a thickness of 6 µm, between a thermosoftening colorant layer and a release layer.

### Example 4

A heat-sensitive recording material was prepared in the same manner as in Example 2, except that a peelable support layer having the following composition was so formed as to have a thickness of 6 µm, between a thermosoftening colorant layer and a release layer.

### Peelable support layer composition

| | |
|---|---|
| Nitrocellulose resin | 95 wt% |
| Ethylene-vinyl acetate copolymer resin | 5 wt% |

By making use of the heat-sensitive recording materials prepared in Examples 3 and 4, the images were formed in the same manner as in Example 1-(4), respectively.

When the resulting recording materials of Examples 3 and 4 were each peeled apart at the peeling angle of 60°, the images remained imagewise on the thermosoftening layers.

### Example 5

A coating solution containing the following thermosoftening colorant layer composition was so coated as to have a coated thickness of 3 g/m², in the same manner as in Example 1, on a flat and smooth sheet of paper forming thereon a thermosoftening layer.

### Thermosoftening colorant layer composition

| | |
|---|---|
| Vinyl chloride-vinyl acetate copolymer | 40 wt% |
| Stearic acid | 40 wt% |
| Nigrosine | 10 wt% |
| Carbon black | 10 wt% |

When an image was printed on the resulting recording material in the same manner as in Example 1, the colorant oozed out of the colorant layer remained imagewise on the thermosoftening layer.

### Example 6

A sample was prepared in the same manner as in Example 5, except that a peelable and anti-fogging layer was arranged by coating the following composition:

The thickness of the anti-fogging layer was 0.5 µm.

### Peelable and anti-fogging layer composition

| | |
|---|---|
| Polyparabanic acid | 80 wt% |
| Stearic acid | 20 wt% |

An image was then formed imagewise in the same manner as in Example 5 with the above-mentioned exception.

### Example 7

A sample was prepared in quite the same manner as in Example 6, except that the following peelable support layer composition was so coated as to have a coated thickness of 6 µm between a thermosoftening colorant layer and a release layer.

### Peeling support layer composition

| | |
|---|---|
| Methyl cellulose | 80 wt% |
| An aqueous dispersion of ethylene-vinyl acetate copolymer | 20 wt% |

An image was then formed imagewise in the same manner as in Examples 5 and 6.

### Example 8

By making use of a 50 µ-thick vinyl chloride resin sheet as a self-supporting type mordant layer, a 6 µm dye-supplying layer comprising the following dye-supplying layer composition was formed on the self-supporting type mordant layer.

On the dye-supplying layer, a 0.3 µm-thick release layer comprising the following release layer forming resin was formed and, thus, a heat-sensitive recording material was obtained so that the self-supporting type mordant layer and the dye-supplying layer may be peeled apart from each other.

### Dye-supplying layer composition

| | |
|---|---|
| Nitrocellulose resin | 70 wt% |
| Dye, MS Cyan VP | 30 wt% |

### Release layer forming resin

| | |
|---|---|
| Silicone-modified urethane resin | 100 wt% |

By making use of a thermal head, heat energy was applied to the resulting heat-sensitive recording material so as to give a printed image. When the self-supporting type mordant layer and the dye-supplying layer were then peeled apart, a sharp and clear printed image was formed on the mordant layer.

### Example 9

Onto a 8-µm thick polyethyleneterephthalate film support, a 10-µm thick adhesive mordant layer comprising the following adhesive mordant layer compositions was formed. And, onto the adhesive mordant layer, a 2-µm thick peelable dye-supplying layer comprising the following dye-supplying layer compositions was formed. Then, onto the dye-supplying layer, a 0.3-µm thick release layer comprising the following release layer forming resin was formed. Thus, a heat-sensitive recording material which was capable of separating the adhesive mordant layer from the dye-supplying layer was prepared.

### Adhesive mordant layer composition

This composition consisted of the polymers compounded of the following monomers:

| | |
|---|---|
| Vinyl chloride | 50 wt% |
| Vinyl acetate | 10 wt% |
| Octyl acrylate | 30 wt% |
| Ethyl acrylate | 5 wt% |
| Anhydrous maleic acid | 5 wt% |

### Dye-supplying layer composition

| | |
|---|---|
| Nitrocellulose resin | 30 wt% |
| Silicone-modified acryl resin | 20 wt% |
| Dye, Kayaset Blue 714 | 30 wt% |
| Silicone resin, polysiloxane resin | 20 wt% |

### Release layer forming resin

| | |
|---|---|
| Silicone-modified acryl resin | 100 wt% |

To the resulting heat-sensitive recording material, heat energy was applied by a thermal head so that a printed image was formed on the adhesive mordant layer.

After heat energy was applied and when the adhesive mordant layer was then separated from the dye-supplying layer, the adhesive mordant layer was so formed as to have a sharp and clear printed image. The adhesive mordant layer may also be used as a label.

### Example 10

On to a 50 µm-thick vinyl chloride resin sheet serving as a self-supporting type mordant layer, a 0.8 µm-thick adhesive layer comprising the following adhesive layer composition was formed: onto the adhesive layer, a 3 µm-thick dye-supplying layer comprising the following dye-supplying layer composition was formed; and a 0.3 µm-thick release layer comprising the following release layer composition was formed; so that a heat-sensitive recording material of which the adhesive layer-attached self-supporting type mordant layer and the dye-supplying layer may be peeled apart from each other could be obtained.

### Adhesive layer composition

The composition consisted of the copolymers compounded of the following monomers:

| | |
|---|---|
| 2-ethyl hexyl | 50 wt% |
| Vinyl acetate | 30 wt% |
| N-tert-butyl acrylate | 20 wt% |

### Dye-supplying layer composition

| | |
|---|---|
| Polyvinyl acetal resin | 70 wt% |
| Dye, MS Yellow VP | 30 wt% |

### Release layer forming resin

| | |
|---|---|
| Silicone-modified urethane resin | 100 wt% |

A printed image was formed on the self-supporting type mordant layer by applying heat energy by a thermal head to the resulting heat-sensitive recording material.

After heat energy was applied and when the adhesive layer attached self-supporting type mordant layer and the dye-supplying layer were then peeled apart from each other, the adhesive layer attached self-supporting type mordant layer was formed with a sharp and clear printed image. The adhesive layer attached self-supporting type mordant layer can also serve as a label.

### Example 11

Onto the surface of a 20-µm thick paper sheet serving as a support, vinyl chloride resin dissolved in a solvent was coated in a thickness of 10 µm so as to serve as a mordant layer. And, onto the surface of the mordant layer, a dye layer comprising nitrocellulose of 80% and Kayaset-Blue-14 dye of 20% dissolved in a solvent was coated in a thickness of 2 µm. Then, onto the surface of the dye layer, polysiloxane resin of 100% was coated to serve as a release layer to be in thickness of 0.5 µm. Thus, a heat-sensitive recording material was prepared.

To the resulting heat-sensitive recording material, heat energy of 40 mj/head was applied imagewise from the release layer side by a serial head.

When the heat energy was applied and the dye layer was then peeled apart from the mordant layer, a beautiful, high-density image was formed on the mordant layer.

### Example 12

Onto one side of a 3.5 µm-thick polyethyleneterephthalate film support, a 0.1 µm-thick release layer comprising silicone-modified urethane resin dissolved in a solvent was coated. And, onto the other side of the support, a 1 µm- thick mordant layer comprising polyester resin dissolved in a solvent was formed. Then, onto the surface of the mordant layer, a 0.5 µm-thick interlayer, i.e., a peeling-antifogging layer, comprising paraffin wax of 80% and polyoxyethylene stearyl ether of 20% each dissolved in a solvent was coated. Further, onto the surface of the inter layer, a 3 µm- thick dye layer comprising polyvinylbutyral of 70% and dye. i.e., MS Magenta-VP, of 30% each dissolved in a solvent was coated. Thus, a heat-sensitive recording material was prepared.

By making use of a line head, heat energy was applied imagewise to the resulting heat-sensitive recording material from the release layer side.

When the heat energy was applied and the mordant layer and the dye layer were then separated from each other, a sharp and clear image was formed on the mordant layer.

## Claims

1. A method of making a heat sensitive transfer recording material for use in a heat sensitive transfer recording system, comprising forming an image receiving layer and providing thereon, a colorant layer containing a colorant and a binder, wherein the image receiving layer is adhered to the colorant layer so firmly that the image receiving layer can be separated from the colorant layer with a peeling force, measured in accordance with JIS 6854, of 0.1 to 1000 g/mm at an angle of 180° after forming an image on the image receiving layer, said method being characterised by comprising
(a) preparing a coating composition comprising said colorant and said binder,
(b) coating said coating composition on to said image receiving layer, and
(c) drying the coated composition to form said colorant layer.

2. The method of claim 1, characterised in that said image receiving layer is a support and said colorant layer is a thermosoftening colorant layer.

3. The method of claim 2, characterised in that the thickness of said support is from 1 to 500 micrometres.

4. The method of claim 1, characterised in that an adhesive layer is provided between said image receiving layer and said colorant layer.

5. The method of claim 4, characterised in that the thickness of the adhesive layer is from 0.1 to 30 micrometres.

6. The method of claim 1, characterised in that the binder comprises a heat-fusible substance or a thermoplastic resin.

7. The method of claim 6, characterised in that said heat-fusible substance includes vegetable wax such as carnauba wax, Japan wax, ouricury wax, and esparto wax; animal wax such as beeswax, insect wax, shellac wax and whale wax; petroleum wax such as paraffin wax, microcrystal wax, polyethylene wax, ester wax and acid wax; mineral wax such as montan wax, ozokerite and ceresin wax; higher aliphatic acids such as palmitic acid, stearic acid, margaric acid and behenic acid; higher alcohols such as palmityl alcohol, stearyl alcohol, behenyl alcohol, margaryl alcohol, myricyl alcohol and eicosanol; higher aliphatic esters such as cetyl palmitate, myricyl palmitate, cetyl stearate and myricyl stearate; amides such as acetamide, propionamide, palmitamide, stearamide and amide wax; higher amines such as stearyl amine, behenyl amine and palmityl amine.

8. The method of claim 6, characterised in that said thermoplastic resin includes ethylene type copolymers, polyacetals, polyamides, polyesters, polyurethanes, polyolefins, polyacrylates, polyvinylchloride, celluloses, rosin, ionomers, petroleum type resins, natural rubber, styrene-butadiene rubber, isoprene rubber, chloroprene rubber, diene type copolymers, ester gum, rosin-maleic resin, rosin-phenol resin, hydrogenated rosin, phenol resin, terpene resin, cyclopentadiene resin and aromatic hydrocarbon type resin.

9. The method of claim 6, characterised in that said thermoplastic resin has a softening point in the range of 50 to 200° C.

10. The method of claim 1, characterised in that said colorant includes organic pigments, inorganic pigments or dyes.

11. The method of claim 2, characterised in that the colorant content of said thermosoftening colorant layer is within the range 5 to 60 per cent by weight.

12. The method of claim 2, characterised in that the thickness of said thermosoftening colorant layer is within the range 0.5 to 20 micrometres.

13. The method of claim 2, characterised in that the material further has a release layer on the outer surface of the thermosoftening colorant layer.

14. The method of claim 13, characterised in that the release layer contains silicone type resins.

15. The method of claim 14, characterised in that the silicone type resin content of the release layer is within the range of 1 to 90 per cent by weight.

16. The method of claim 13, characterised in that the thickness of the release layer is from 0.03 to 30 micrometres.

17. The method of claim 1, characterised in that said colorant layer is a dye-supplying layer.

18. The method of claim 17, characterised in that said colorant layer contains a thermally diffusing dye.

19. The method of claim 18, characterised in that said dye has a molecular weight from 50 to 4000.

20. The method of claim 18, characterised in that the melting point, sublimation temperature or vaporizing temperature of said dye is within the range of 60 to 300° C.

21. The method of claim 18, characterised in that the dye content of said colorant layer is within the range of 5 to 80 per cent by weight.

22. The method of claim 17, characterised in that the thickness of the dye-supplying layer is from 0.5 to 30 micrometres.

23. The method of claim 1, characterised in that said image-receiving layer contains an adhesive composition.

24. The method of claim 1, characterised in that said colorant layer contains an adhesive composition.

25. The method of claim 1, characterised in that a transparent support is provided on the outer surface of the image receiving layer.

26. The method of claim 1, characterised in that a peelable layer containing at least one selected from the group consisting of silicone resin, silicone-modified resin, wax and a surfactant is provided between said image receiving layer and said colorant layer.

27. The method of claim 26, characterised in that the thickness of said peelable layer is from 0.1 to 10 micrometres.

28. The method of claim 1, characterised in that an anti-fogging layer containing at least one selected from the group consisting of a thermoplastic resin, heat-fusible substance and a filler is provided between said image receiving layer and said colorant layer.

29. The method of claim 28, characterised in that the thickness of said anti-fogging layer is form 0.3 to 10 micrometres.

30. The method of claim 1, characterised in that the material further comprises a peelable support layer on the outer surface of the colorant layer.

31. The method of claim 30, characterised in that said peelable support layer is composed of at least one selected from the group consisting of polyacrylate resins, cellulose resins, polycarbonate resins and polyparabanic acid resin.

## Patentansprüche

1. Verfahren zur Herstellung eines wärmeempfindlichen Übertragungsaufzeichnungsmaterials für den Einsatz bei einem wärmeempfindlichen Übertragungsaufzeichnungssystem, das darin besteht, daß man eine Bildempfangsschicht herstellt und darauf eine Farbmittelschicht aufbringt, die ein Farbmittel und ein Bindemittel enthält, wobei die Bildempfangsschicht so fest an der Farbmittelschicht haftet, daß sich die Bildempfangsschicht nach Erzeugen eines Bildes auf der Bildempfangsschicht von der Farbmittelschicht bei einer gemäß JIS 6854 gemessenen Schälkraft von 0,1 bis 1000 g/mm bei einem Winkel von 180° abziehen läßt, wobei das Verfahren dadurch gekennzeichnet ist, daß man zur Herstellung der Farbmittelschicht
(a) eine Überzugszusammensetzung aus dem Farbmittel und dem Bindemittel herstellt,
(b) die Bildempfangsschicht mit der Überzugszusammensetzung beschichtet und
(c) die aufgetragene Zusammensetzung trocknet.

2. Verfahren nach Anspruch 1, dadurch gekennzeichnet, daß es sich bei der Bildempfangsschicht um einen Träger und bei der Farbmittelschicht um eine Schicht aus einem thermisch erweichenden Farbmittel handelt.

3. Verfahren nach Anspruch 2, dadurch gekennzeichnet, daß die Dicke des Trägers 1 bis 500 µm beträgt.

4. Verfahren nach Anspruch 1, dadurch gekennzeichnet, daß zwischen der Bildempfangsschicht und der Farbmittelschicht eine Haftschicht angeordnet ist.

5. Verfahren nach Anspruch 4, dadurch gekennzeichnet, daß die Dicke der Haftschicht 0,1 bis 30 µm beträgt.

6. Verfahren nach Anspruch 1, dadurch gekennzeichnet, daß das Bindemittel aus einer wärmeschmelzbaren Substanz oder einem Thermoplastharz besteht.

7. Verfahren nach Anspruch 6, dadurch gekennzeichnet, daß als wärmeschmelzbare Substanz Pflanzenwachs wie Karnaubawachs, Japanwachs, Ouricurywachs und Espartowachs, tierisches Wachs wie Bienenwachs, Insektenwachs, Schellackwachs und Walwachs, Erdölwachs wie Paraffinwachs, Mikrowachs, Polyethylenwachs, Esterwachs und Säurewachs, Mineralwachs wie Montanwachs, Ozokerit- und Ceresinwachs, höhere aliphatische Säuren wie Palmitinsäure, Stearinsäure, Margarinsäure und Behensäure, höhere Alkohole wie Palmitylalkohol, Stearylalkohol, Behenylalkohol, Margarylalkohol, Myricylalkohol und Eicosanol, höhere aliphatische Ester wie Palmitinsäure-cetylester, Palmitinsäure-myricylester, Stearinsäure-cetylester und Stearinsäure-myricylester, Amide wie Acetamid, Propionamid, Palmitamid, Stearamid und Amidwachs, höhere Amine wie Stearylamin, Behenylamin und Palmitylamin in Frage kommen.

8. Verfahren nach Anspruch 6, dadurch gekennzeichnet, daß als Thermoplastharz Copolymere des Ethylentyps, Polyacetale, Polyamide, Polyester, Polyurethane, Polyolefine, Polyacrylate, Polyvinylchlorid, Cellulosen, Kolophonium, Ionomere, Harze des Erdöltyps, Naturkautschuk, Styrol-Butadien-Kautschuk, Isoprenkautschuk, Chloroprenkautschuk, Copolymere des Dientyps, Esterharz, Kolophonium-Malein-Harz, Kolophonium-Phenol-Harz, hydriertes Kolophonium, Phenolharz, Terpenharz, Cyclopentadienharz und Harze vom Typ aromatischer Kohlenwasserstoffe in Frage kommen.

9. Verfahren nach Anspruch 6, dadurch gekennzeichnet, daß das Thermoplastharz einen Erweichungspunkt im Bereich von 50 bis 200°C besitzt.

10. Verfahren nach Anspruch 1, dadurch gekennzeichnet, daß als Farbmittel organische Pigmente, anorganische Pigmente oder Farbstoffe in Frage kommen.

11. Verfahren nach Anspruch 2, dadurch gekennzeichnet, daß der Farbmittelgehalt der Schicht aus thermisch erweichendem Farbmittel im Bereich von 5 bis 60 Gew.-% liegt.

12. Verfahren nach Anspruch 2, dadurch gekennzeichnet, daß die Dicke der Schicht aus thermisch erweichendem Farbmittel im Bereich von 0,5 bis 20 µm liegt.

13. Verfahren nach Anspruch 2, dadurch gekennzeichnet, daß das Material auf der Außenfläche der Schicht aus thermisch erweichendem Farbmittel weiterhin eine Trennschicht aufweist.

14. Verfahren nach Anspruch 13, dadurch gekennzeichnet, daß die Trennschicht Harze des Silikontyps enthält.

15. Verfahren nach Anspruch 14, dadurch gekennzeichnet, daß der Gehalt der Trennschicht an Harzen des Silikontyps im Bereich von 1 bis 90 Gew.-% liegt.

16. Verfahren nach Anspruch 13, dadurch gekennzeichnet, daß die Dicke der Trennschicht 0,03 bis 30 µm beträgt.

17. Verfahren nach Anspruch 1, dadurch gekennzeichnet, daß die Farbmittelschicht eine farbstoffliefernde Schicht ist.

18. Verfahren nach Anspruch 17, dadurch gekennzeichnet, daß die Farbmittelschicht einen thermisch diffundierenden Farbstoff enthält.

19. Verfahren nach Anspruch 18, dadurch gekennzeichnet, daß der Farbstoff ein Molekulargewicht von 50 bis 4000 besitzt.

20. Verfahren nach Anspruch 18, dadurch gekennzeichnet, daß der Schmelzpunkt, die Sublimationstemperatur oder die Verdampfungstemperatur des Farbstoffs im Bereich von 60 bis 300°C liegt.

21. Verfahren nach Anspruch 18, dadurch gekennzeichnet, daß der Farbstoffgehalt der Farbmittelschicht im Bereich von 5 bis 80 Gew.-% liegt.

22. Verfahren nach Anspruch 17, dadurch gekennzeichnet, daß die Dicke der farbstoffliefernden Schicht 0,5 bis 30 µm beträgt.

23. Verfahren nach Anspruch 1, dadurch gekennzeichnet, daß die Bildempfangsschicht eine Klebstoffzusammensetzung enthält.

24. Verfahren nach Anspruch 1, dadurch gekennzeichnet, daß die Farbmittelschicht eine Klebstoffzusammensetzung enthält.

25. Verfahren nach Anspruch 1, dadurch gekennzeichnet, daß auf der Außenfläche der Bildempfangsschicht ein transparenter Träger angeordnet ist.

26. Verfahren nach Anspruch 1, dadurch gekennzeichnet, daß zwischen der Bildempfangsschicht und der Farbmittelschicht eine abziehbare Schicht angebracht ist, die zumindest eine aus der Gruppe Silikonharz, mit Silikon modifiziertes Harz, Wachs und Tensid ausgewählte Substanz enthält.

27. Verfahren nach Anspruch 26, dadurch gekennzeichnet, daß die Dicke der abziehbaren Schicht 0,1 bis 10 µm beträgt.

28. Verfahren nach Anspruch 1, dadurch gekennzeichnet, daß zwischen der Bildempfangsschicht und der Farbmittelschicht eine schleierverhütende Schicht angebracht ist, die zumindest eine aus der Gruppe Thermoplastharz, wärmeschmelzbare Substanz und Füllmittel ausgewählte Substanz enthält.

29. Verfahren nach Anspruch 28, dadurch gekennzeichnet, daß die Dicke der schleierverhütenden Schicht 0,3 bis 10 µm beträgt.

30. Verfahren nach Anspruch 1, dadurch gekennzeichnet, daß das Material auf der Außenfläche der Farbmittelschicht weiterhin eine abziehbare Trägerschicht aufweist.

31. Verfahren nach Anspruch 30, dadurch gekennzeichnet, daß die abziehbare Trägerschicht aus mindestens einer aus der Gruppe der Polyacrylatharze, Celluloseharze, Polycarbonatharze und Polyparabansäureharz ausgewählten Substanz besteht.

## Revendications

1. Méthode pour la fabrication d'un matériau d'enregistrement par transfert thermique pour utilisation dans un système d'enregistrement par transfert thermique, comprenant la formation d'une couche de réception d'image et la fourniture sur celle-ci d'une couche de colorant contenant un colorant et un liant, dans laquelle la couche de réception d'image adhère à la couche de colorant de manière si ferme que la couche de réception d'image peut être séparée de la couche de colorant avec une force de pelage, mesurée conformément à la norme JIS 6854, de 0,1 à 1000 g/mm à un angle de 180° après la formation d'une image sur la couche de réception d'image, ladite méthode étant caractérisée en ce qu'elle comprend
(a) la préparation d'une composition de revêtement comprenant ledit colorant et ledit liant,
(b) le revêtement de ladite composition de revêtement sur ladite couche de réception d'image, et
(c) le séchage de la composition revêtue pour former ladite couche de colorant.

2. Méthode de la revendication 1, caractérisée en ce que ladite couche de réception d'image est un support et en ce que ladite couche de colorant est une couche de colorant à ramollissement thermique.

3. Méthode de la revendication 2, caractérisée en ce que l'épaisseur dudit support est de 1 à 500 micromètres.

4. Méthode de la revendication 1, caractérisée en ce que l'on prévoit une couche adhésive entre ladite couche de réception d'image et ladite couche de colorant.

5. Méthode de la revendication 4, caractérisée en ce que l'épaisseur de la couche adhésive est de 0,1 à 30 micromètres.

6. Méthode de la revendication 1, caractérisée en ce que le liant comprend une substance thermofusible ou une résine thermoplastique.

7. Méthode de la revendication 6, caractérisée en ce que ladite substance thermofusible inclut de la cire végétale telle que la cire de carnauba, la cire du Japon, la cire d'ouricury et la cire d'alfa; de la cire animale telle que la cire d'abeilles, la cire d'insectes, la cire shellac et la cire de baleine; de la cire de pétrole telle que la cire de paraffines, la cire microcristalline, la cire de polyéthylène, la cire d'esters et la cire d'acide; de la cire minérale telle que la cire montanique, la cire fossile et la cire cérésine; des acides aliphatiques supérieurs tels que l'acide palmitique, l'acide stéarique, l'acide margarique et l'acide béhénique; des alcools supérieurs tels que l'alcool palmitylique, l'alcool stéarylique, l'alcool béhénylique, l'alcool margarylique, l'alcool myricylique et l'eicosanol; des esters aliphatiques supérieurs tels que le palmitate de cétyle, le palmitate de myricyle, le stéarate de cétyle et le stéarate de myricyle; des amides tels que l'acétamide, le propionamide, le palmitamide, le stéaratamide et la cire d'amide; des amines supérieures telles que l'amine stéarylique, l'amine béhénylique, et l'amine palmitylique.

8. Méthode de la revendication 6, caractérisée en ce que ladite résine thermoplastique inclut des copolymères du type éthylène, des polyacétals, des polyamides, des polyesters, des polyuréthanes, des polyoléfines, des polyacrylates, du chlorure de polyvinyle, des celluloses, la résine de pin, des ionomères, des résines du type pétrole, le caoutchouc naturel, le caoutchouc styrène-butadiène, le caoutchouc isoprène, le caoutchouc chloroprène, des copolymères du type diénique, l'ester de colophane, la résine maléique-résine de pin, la résine de pin-phénol, la résine de pin hydrogénée, la résine phénolique, la résine terpénique, la résine cyclopentadiénique et la résine du type hydrocarbures aromatiques.

9. Méthode de la revendication 6, caractérisée en ce que ladite résine thermoplastique a un point de ramollissement dans le domaine de 50 à 200°C.

10. Méthode de la revendication 1, caractérisée en ce que ledit colorant inclut des pigments organiques, des pigments minéraux ou des matières tinctoriales.

11. Méthode de la revendication 2, caractérisée en ce que la teneur en colorant dudit colorant à ramollissement thermique est dans le domaine de 5 à 60 % en poids.

12. Méthode de la revendication 2, caractérisée en ce que l'épaisseur de la couche de colorant à ramollissement thermique est dans le domaine de 0,5 à 20 micromètres.

13. Méthode de la revendication 2, caractérisée en ce que le matériau a en outre une couche de séparation sur la surface externe de la couche de colorant à ramollissement thermique.

14. Méthode de la revendication 13, caractérisée en ce que la couche de séparation contient des résines du type silicones.

15. Méthode de la revendication 14, caractérisée en ce que la teneur en résine du type silicones de la couche de séparation est dans le domaine de 1 à 90 % en poids.

16. Méthode de la revendication 13, caractérisée en ce que l'épaisseur de la couche de séparation est de 0,03 à 30 micromètres.

17. Méthode de la revendication 1, caractérisée en ce que ladite couche de colorant est une couche fournissant la matière tinctoriale.

18. Méthode de la revendication 17, caractérisée en ce que ladite couche de colorant contient une matière tinctoriale à diffusion thermique.

19. Méthode de la revendication 18, caractérisée en ce que ladite matière tinctoriale a un poids moléculaire de 50 à 4 000.

20. Méthode de la revendication 18, caractérisée en ce que le point de fusion, la température de sublimation ou la température de vaporisation de ladite matière tinctoriale est dans le domaine de 60 à 300°C.

21. Méthode de la revendication 18, caractérisée en ce que la teneur en matière tinctoriale de ladite couche de colorant est dans le domaine de 5 à 80 % en poids.

22. Méthode de la revendication 17, caractérisée en ce que l'épaisseur de la couche fournissant la matière tinctoriale est de 0,5 à 30 micromètres.

23. Méthode de la revendication 1, caractérisée en ce que ladite couche de réception d'image contient une composition adhésive.

24. Méthode de la revendication 1, caractérisée en ce que ladite couche de colorant contient une composition adhésive.

25. Méthode de la revendication 1, caractérisée en ce que l'on prévoit un support transparent sur la surface externe de la couche de réception d'image.

26. Méthode de la revendication 1, caractérisée en ce que l'on prévoit une couche que l'on peut peler, contenant au moins un produit choisi parmi le groupe se composant d'une résine de silicones, d'une résine modifiée aux silicones, d'une cire et d'un agent tensioactif, entre ladite couche de réception d'image et ladite couche de colorant.

27. Méthode de la revendication 26, caractérisée en ce que l'épaisseur de ladite couche que l'on peut peler est de 0,1 à 10 micromètres.

28. Méthode de la revendication 1, caractérisée en ce que l'on prévoit une couche anti-voilage contenant au moins un produit choisi parmi le groupe se composant d'une résine thermoplastique, d'une substance thermofusible et d'une charge, entre ladite couche de réception d'image et ladite couche de colorant.

29. Méthode de la revendication 28, caractérisée en ce que l'épaisseur de ladite couche anti-voilage est de 0,3 à 10 micromètres.

30. Méthode de la revendication 1, caractérisée en ce que le matériau comprend en outre une couche de support que l'on peut peler sur la surface externe de la couche de colorant.

31. Méthode de la revendication 30, caractérisée en ce que ladite couche de support que l'on peut peler est composée d'au moins un produit choisi parmi le groupe se composant des résines polyacrylates, des résines cellulosiques, des résines polycarbonates et de la résine d'acide polyparabanique.
